

# UNITED STATES PATENT OFFICE.

WILLIAM BECKERS AND ISAAC DREYFUS, OF BROOKLYN, NEW YORK, ASSIGNEES TO  
W. BECKERS ANILINE AND CHEMICAL WORKS, OF BROOKLYN, NEW YORK.

## CHROMIUM COMPOUND.

1,162,210.

Specification of Letters Patent. Patented Nov. 30, 1915.

No Drawing.

Application filed March 24, 1914. Serial No. 826,944.

To all whom it may concern:

Be it known that we, WILLIAM BECKERS and ISAAC DREYFUS, both citizens of the United States, and residents of the borough of Brooklyn, in the county of Kings, city and State of New York, have invented certain new and useful Improvements in Chromium Compounds, of which the following is a specification.

10 The object of our invention is a method for the production of new, novel and useful chromium compounds the aqueous solutions of which are not precipitable by means of alkalis or mordant colors and for the products produced thereby. Whereas, chromium compounds may be easily precipitated from their aqueous solutions by means of alkalis or mordant colors, we have found that it is possible to produce a chromium compound 15 under such circumstances and conditions that the chromium compound contained therein is not precipitated from its aqueous solution by the alkalis or mordant colors. The solutions thus produced remain perfectly 20 clear and unprecipitated even when boiled with alkali hydrates or with the mordant colors and possess mordanting properties in dyeing of great commercial value.

25 If a solution of a neutral chromate compound of an alkali-metal be added to glucose and heated until no chromic acid can be detected by means of an acidulated potassium iodid solution, the resulting product is a solution of a chromium compound in such 30 physical and chemical condition that no precipitate is formed upon the addition of alkalis such as sodium carbonate, potassium carbonate, sodium hydrate, potassium hydrate, etc., or upon the addition of mordant colors 35 such as alizarin, logwood, etc. While the exact composition of these solutions has not been definitely determined, it would seem that the chromium compounds are present in a colloidal form preventing their precipitation. This solution has the property of 40 forming chromium lakes of the mordant colors which are completely soluble in the solution and which do not precipitate upon continued standing. This property gives 45 the solution great value in the dyeing industry.

50 When the ordinary solution of a chromium compound is added to a solution of a mordant color such as the alizarins, logwood,

etc., and heated, an insoluble precipitate is 55 at once formed and it is the formation of this color lake on the fiber that gives these dyestuffs their commercial value in the dyeing industry.

Successful dyeing of textile fibers with 60 the mordant colors presents many difficulties and requires great care and the observance of cautions in the application of the dyeing methods employed. The usual 65 methods of dyeing with these colors is to first mordant the fiber with a chromium compound and then subject it to a solution of the dyestuff, or to reverse the operation and treat the fiber first with the dyestuff 70 and then with the chromium mordant. This 75 requires a number of steps in the dyeing operation and it is evident that unless the fiber is thoroughly penetrated with each solution and the excess liquor carefully removed from the fiber after each step, the resulting dyeings will be unsatisfactory. It 80 will thus be seen that on account of the insoluble-lake-forming properties of these colors, they are liable to accumulate upon the surface of the fiber, causing uneven dyeings, non-penetration, and results which 85 crock and are not fast to washing, scouring and the other ordinary operations to which such goods are subjected.

It is evident that if a perfectly clear solution of the chromium compound, or a perfectly clear solution of the chromium compound and the dyestuff can be formed and the textile fiber be thoroughly saturated or 90 penetrated with this solution and the insoluble lake be produced within the fiber, after its penetration by this solution, the resulting dyeings will be more uniform and more thoroughly incorporated throughout the fiber, and that they will not have a 95 tendency to crock and will be faster to the various operations to which the goods are subjected. We have found that the solutions formed by our new method have these 100 properties and hence possess great value for the dyeing of textile fibers. The following example represents one method of following our invention: dissolve 108 pounds of glucose in 216 pounds water and gradually add 55 pounds neutral chromate of sodium 105 with constant stirring, maintaining a temperature of 80 degrees to 90 degrees C. Heat until the presence of chromic acid

cannot be detected by an acidulated solution of potassium iodid. The whole operation generally requires from two to three hours. Neutralize with acetic acid which requires about 20 pounds acetic acid 70 per cent. If a solution of mordant colors or mordant-forming dyes such as the alizarins, logwood, etc., be added to this solution a perfectly clear solution of the chromium compound of the dyestuff is formed which retains its solubility even upon boiling or upon long standing. If the solution thus formed be carefully evaporated to dryness, as for instance upon a water-bath, there results a dry brittle product, which when dissolved in water possesses all of the properties described herein for the solution before evaporation.

We do not limit ourselves to the particular ingredients, the quantities, times or temperatures mentioned above, nor to the particular order of the incorporation of the ingredients, all of which may be varied without going beyond the scope of our invention as described and claimed.

What is claimed, is:

1. The process of treating glucose and neutral chromium compounds comprising heating them together in solution, thereby producing a solution of a chromium compound not precipitable by alkalis or mordant colors.
2. The process of treating glucose and neutral chromates of alkali-metals comprising heating them together in solution, thereby producing a solution of a chromium compound not precipitable by alkalis or mordant colors and evaporating to dryness.
3. The process of treating glucose and neutral chromate of soda comprising heating them together in solution, thereby producing a solution of a chromium compound not

precipitable by alkalis or mordant colors and evaporating to dryness.

4. As a new article of manufacture, a chromium compound producible by treating glucose and a neutral chromium compound from the aqueous solution of which the produced chromium compound is not precipitable by alkalis or mordant colors. 45

5. As a new article of manufacture, a chromium compound producible by treating glucose and a neutral chromate of an alkali-metal from the aqueous solution of which the produced chromium compound is not precipitable by alkalis or mordant colors. 50

6. As a new article of manufacture, a chromium compound producible by treating glucose and a neutral chromate of soda from the aqueous solution of which the produced chromium compound is not precipitable by alkalis or mordant colors. 60

7. A dry brittle product producible by adding a neutral chromate of an alkali-metal to a solution of glucose, heating and evaporating to dryness, from the aqueous solution of which the produced chromium compound is not precipitable by alkalis or mordant colors. 65

8. A dry brittle product producible by adding neutral chromate of soda to a solution of glucose, heating and evaporating to dryness, from the aqueous solution of which the produced chromium compound is not precipitable by alkalis or mordant colors. 70

Signed at the borough of Brooklyn, in the county of Kings, city and State of New York, this 21st day of March, 1914.

WILLIAM BECKERS.  
ISAAC DREYFUS.

Witnesses:

S. R. DAVID,  
I. KOR FIEXE.